

## UNITED STATES PATENT OFFICE

2,212,369

## SYNTHETIC OIL FOR TREATING TEXTILES

Alphons O. Jaeger, Mount Lebanon, Pa., assignor to American Cyanamid & Chemical Corporation, New York, N. Y., a corporation of Delaware

No Drawing. Application January 14, 1938,  
Serial No. 184,931

5 Claims. (Cl. 252—57)

This invention relates to the oiling or lubrication of textile filaments, threads or fabrics such as woolens, worsteds, silk, cotton and artificial fibers such as cellulose acetate, rayon, 5 viscose, regenerated cellulose and the like and more particularly to a new class of lubricants for use in such oiling or lubrication.

Heretofore the materials generally called lubricants which have been used for the above 10 purposes were of natural, and usually of animal or vegetable origin. For the worsteds olive oil has been the principal lubricant while for woolens and low woolens a mixture of such oils as olive oil, 15 teaseed oil or "oleins," which are crude oleic acids containing a high percentage of free fatty acid, have been used. In many cases these oils have been mixed with mineral oils, the latter being present in amounts of 10—20% by weight or more.

The many limitations of these natural oils and 20 oil mixtures have long been recognized in the textile trade, but no substitute as yet proposed has been fully satisfactory. It is true that proposals have been made to use glycerol, or to improve the scouring properties by reacting 25 triglycerides such as olive oil or coconut oil with sufficient amounts of glycerol to produce the monoglyceride but these modified oils and fats still retain the disadvantages characteristic of the natural oils themselves.

30 I have now found that lubricants for textiles of the above types are greatly improved when they contain or consist of esters of organic polycarboxylic acids or their anhydrides with a monohydric or polyhydric alcohol, or combined esters 35 thereof. Many of the synthetic chemical compounds of this class are excellent lubricants when used singly or in admixture with each other as a synthetic textile oil, but it is a characteristic property of all the members of this class of materials that they will improve any of the materials of natural origin now used as lubricating agents when mixed with them in substantial quantities.

Accordingly, my invention comprises a process 40 of lubricating textiles or textile fibers by the application thereto of lubricants consisting of or containing synthetic esters of the above defined class, either singly or in admixture. A further object of the invention resides in the improvement of the lubricating, scouring or other properties of textile lubricants by the incorporation 45 therein of unmodified or modified esters of organic polycarboxylic acids. A still further object of the invention resides in the improvement 50 of lubricants for textiles by decreasing or

eliminating their capacity for spontaneous combustion and increasing their fluidity at low temperatures, these improvements being characteristic of textile lubricants consisting of or containing substantial quantities of the unmodified or modified esters of organic polycarboxylic acids with monohydric or polyhydric alcohols of the present invention.

The polycarboxylic acids which may be employed in preparing esters for use in accordance with the present invention may be aliphatic, hydroaromatic or aromatic, but I have also found that the esters of the aromatic and hydroaromatic polycarboxylic acids have in general better qualities than have the esters of aliphatic polycarboxylic acids. However, esters of aliphatic dicarboxylic acids are also useful, particularly as agents for improving the scouring value of the lubricants, and to this extent they are also included within the scope of the invention. For 10 example, I have found that the class of aliphatic dicarboxylic acids consisting of maleic acid, its isomer fumaric acid and its reduction product succinic acid will produce esters which have excellent scouring properties for textiles fibers, and the ester of the sulfonated or phosphorylated acids of this class are even better. Moreover, esters of the aliphatic acids may be used to modify 15 certain of the characteristics of the aromatic and hydroaromatic dicarboxylic acid esters of polyhydric alcohols, as will be subsequently explained, and the esters of this class are therefore also included within the scope of the invention.

Among the aromatic di- and polycarboxylic acids whose esters form the preferred lubricating 20 agents of the present invention phthalic acid or anhydride and its modification products such as sulfophthalic and halogenated phthalic acids such as the chlorophthalic acids occupy an outstanding position by reason of their commercial availability and relatively low price and the low vapor pressure and excellent lubricating qualities of their esters. Among the di- and polycarboxylic acids of the hydroaromatic series, those obtainable by the selective hydrogenation of 25 phthalic acid and by the diene synthesis are of greatest interest since they produce low vapor pressure esters of excellent stability having good lubricating properties for textile fibers.

The alcohols or other esterifying agents which 30 can be used in preparing the esters which form the preferred lubricants for textiles in accordance with the present invention may be selected from a wide range of compounds. Any monohydric alcohol of the paraffin series may be used,

such as ethyl, methyl, propyl, butyl, amyl, hexyl, heptyl or octyl alcohols such as cetyl alcohol, ethyl hexyl alcohol, etc. as well as the corresponding higher alcohols from the saponification of 5 waxes and the reduction of fatty acids such as lauryl alcohol, palmityl alcohol, ceryl alcohol, etc. In addition to the straight chain alcohols, isomeric or branched chain alcohols may be used, including such compounds as isopropyl alcohol, 10 isobutyl alcohol, isobutyl carbinol or other isobutyl alcohols, capryl alcohol, pinacolyl alcohol, tetramethyl-ethyl or other isomeric hexyl alcohols and the like as well as higher alcohols of 15 this nature. Another class of alcohols which are 15 of value in producing esters for use in the textile lubrication are ether alcohols such as methoxy, ethoxy and butoxy ethanols, aromatic ether alcohols such as phenoxyethanols, alkyl phenoxyethanols, etc.

20 In addition to the saturated monohydric alcohols, the corresponding alcohols of the olefin series may be used. Allyl and crotonyl alcohols are typical lower alcohols of this type which may be employed in some cases and oleyl alcohol is a 25 typical higher alcohol. Mixed alcohols from special sources may also be used, such as the mixture of isomeric amyl alcohols obtainable from the absorption in sulfuric acid and subsequent hydrolysis of casing head gas or other petroleum 30 fractions and sold as "Pentasol"; mixed alcohols from similar treatment of other petroleum fractions; synthetic lower and higher alcohols from the catalytic reduction of carbon monoxide or dioxide or from the hydrogenation of coal and 35 oils, etc.

Another important class of alcohols which may be used in preparing esters for textile lubrication are those of a cyclic nature such as the aromatic alcohols including benzyl alcohol, the tolyl carbinols, the naphthyl carbinols, dialkyl benzyl alcohols and the like. Esters of these alcohols are particularly valuable for admixture with lubricating oils of natural origin, such as olive oil, castor oil, teaseed oil and the like, by reason of their anti-45 oxidant properties. Another special type of compounds falling within this classification are the inner esters, the lactones, which may be produced for example by reduction of polybasic acids having at least two carboxyl groups in ortho position. 50 Phthalide, which is a reduction product of phthalic anhydride, is an example of such a lactone. I have found that this compound may be incorporated to advantage in lubricants for textile fibers, especially in combination with esters of 55 organic dicarboxylic acids. Other lactones such as those obtainable by partial reduction of hydroaromatic acids resulting from the diene synthesis may also be used, a typical example of such acids being the condensation product of maleic or fumaric acid with rosin or with dehydrated castor oil, linseed oil or the fatty acids thereof. Corresponding ester products of such acids as contain 60 free carboxyl groups may also be used. Hydrogenation and substitution products of the above 65 compounds may also be used such as hydrogenated and substituted phthalides, these derivatives having physical properties which vary with the degree of hydrogenation and substitution and offer in themselves a wide field of choice for the 70 purposes of the present invention. Other alcohols and acids may also be used, for example mono- or polyhydroxy organic acids containing one or more carboxyl groups, in which acids one or more of the hydroxy groups may be esterified 75 with a polycarboxylic acid.

It is understood that any of the esters which may be prepared by esterification of the above alcohols, either singly or in admixture, with polycarboxylic acids may be used in the oiling of textiles. These esters are well suited for use as the sole treating agent in these processes, but another important feature of the invention resides in their use in conjunction with the vegetable or animal oils, mineral oils, fats and fatty acids which are now used for these purposes. This is important, 10 not only by reason of the wider field of choice which is made available by the use of a mixture of lubricants, but also because the long experience which has already been acquired in treating textiles with natural oils and fatty acids becomes 15 available in applying the mixtures thereof with the esters of the present invention. When synthetic esters are used in conjunction with the natural oils and fats, their relative stability and the greater lubricating properties which many of 20 them possess will result in improvements without substantial modification of the methods of application now in use, and this constitutes an important advantage of the invention.

Another advantage flowing from the use of 25 esters of phthalic acid in conjunction with the natural oils and fats now used for technical lubrication is the resistance of these esters to ultraviolet light. The incorporation of even small 30 quantities of any of the above described phthalic acid compounds into the oiling compositions now used for textiles will result in an increased stability against rancidity and spontaneous combustion and will produce more even dyeings in the 35 finished textiles.

Another feature of the invention which is of great practical importance resides in the modification of the synthetic esters of the present invention by the introduction of the inorganic or 40 organic substituents. For example, the sulfonation of these esters or the use of sulfonated acids or sulfonated alcohols in their preparation results in a lubricant which is more easily emulsified and more easily removed from the finished goods by the ordinary detergents now in use, and 45 the introduction of amino, halogen, hydroxy and similar groups also will impart special properties. The most important products of this nature are, of course, sulfonation products; and these may be prepared by any of the known sulfonation 50 processes. A particularly useful method of applying this feature of the invention is the partial sulfonation of the completed ester, or the use of a mixture of sulfonated and unsulfonated acids in esterifying, whereby an incompletely sulfonated 55 product is produced. This method permits the preparation of textile oils having not only good lubricating characteristics but having exactly the right emulsification properties for proper removal after weaving of the fabrics and, 60 in fact, the use of esters of a mixture of sulfonated and unsulfonated acids will in many cases produce a composition which requires no additional detergent for removal. For example, a mixture of 90 parts by weight of dimethyl phthalate and 10 parts of the sodium salt of diethyl sulfosuccinate or diethyl sulfophthalate constitutes a satisfactory lubricant for woolen fibers that can easily be removed by simple agitation in hot water.

In addition to the esters of organic dicarboxylic 70 acids with monohydric alcohols of the classes enumerated, there are certain classes of reaction products of these acids with dihydric and polyhydric alcohols and their ether compounds which are of value in the lubrication of textiles, and 75

which are included in the invention. Many of the esters of this class, such as the phthalic glycerides, harden or polymerize to synthetic resins which in themselves have no lubricating value, but I have found that many of the esters of this class may be modified in such a manner as to produce liquids of relatively low viscosity having excellent lubricating properties. For example, the reaction products of polyhydric alcohols with organic dibasic acids, which reaction products contain substantial quantities of oils or oily materials such as higher fatty acids as modifying agents, with or without additional esterification with monohydric alcohols, form excellent lubricants for textiles.

Another advantage of esters of polyhydric alcohols with polybasic acids is the opportunity which they present for preparing compounds containing an excess of hydroxy groups over and above those necessary for esterification of the polycarboxylic acids themselves. I have found, as an important feature of the invention, that esters of polyhydric alcohols with polybasic acids, which esters contain an excess of hydroxy or ether groups as above defined have important scouring properties and are much more easily removed from the fiber by the ordinary detergent after spinning and weaving. These hydroxy groups may be present in uncombined form, as in the case of diglycol phthalate, phthalate, dibenzoyl diglyceryl maleate, etc., or they may be completely esterified with monobasic acids as in the case of dioleyl diglycol monophthalate, or succinate. The results obtainable with combining examples of this class are illustrated in the following examples.

Suitable oils, fats or fatty acids which may be used for modifying polyhydric alcohol esters of polybasic acids for textile lubricants include the non-drying vegetable oils, such as cottonseed oil, palm oil, corn oil, coconut oil, olive oil, teaseed oil, etc., animal oils and the like, either singly or in admixture. Frequently it is of advantage to use the fatty acids obtained by the hydrolysis of these or other oils, which fatty acids are non-drying, i. e. which are obtained from fats or oils having an iodine value not greatly in excess of 100 and do not polymerize to a greater extent than does castor oil on blowing with air. A special class of acids which are readily obtainable and are excellently suitable for this purpose are the fatty acids such as oleic and stearic acids derived from taloil or black liquor soap which is produced as by-product in the kraft process of paper pulp manufacture.

The compounds obtained upon introduction of the above oils, fats, and fatty acids into complex esters of polybasic acids with polyhydric alcohols may be further modified by combination with any of the monohydric alcohols, such as those previously described, or by combination with non-oil acids such as benzoic acid, acetic acid, furoic acid, propionic acid, tetrahydrobenzoic acid, etc. This class of compounds is known technically by the term "long oil alkyl resins," which term is defined as a polyhydric alcohol-poly-carboxylic acid ester containing at least 50% of an oil or of a fatty acid obtained from an oil.

The lubricants of the present invention may be applied to the textiles by any of the methods now in use, and may be employed as such, in admixture with each other, in the form of emulsions, or in admixture with soaps in the form of the so-called wool creams. Irrespective of the method of application, however, it is an advan-

tage of the present invention that all the synthetic esters used therein are readily emulsifiable with most of the emulsifying and scouring agents now used in the wool industry, which greatly facilitates their removal from the fiber after weaving or knitting. A short list of surface active agents which may be used in preparing the lubricants in emulsified form or for removing them from the finished piece goods is the following.

(1) Sulfonated aromatic hydrocarbons and their homologs, such as sulfonated naphthalene, propyl or isopropyl, butyl or isobutyl and amyl naphthalene sulfonic acids, or their ammonium, alkali metal or triethanol amine salts.

(2) Salts of sulfonated aromatic or aliphatic esters of mono-, di- and polycarboxylic acids, such as dipropyl, diethyl, di-(methyl amyl) or di-octyl esters of sulfonated phthalic acid.

(3) Sulfated or sulfonated higher alcohols, such as sulfonated lauryl or other alcohols prepared from the fatty acids of vegetable oils.

(4) Sulfonated mineral, vegetable or animal oils such as the "quasols" which are castor oils of varying degrees of sulfonation.

(5) Sulfonated amides and imides of aromatic or aliphatic, mono-, di- and polycarboxylic acids.

(6) Salts of diene condensation products, such as the sodium, ammonium or triethanolamine salts of the condensation products of abietic and maleic or fumaric acids and their esters, salts and sulfonation products.

(7) Soaps of various fatty acids such as oleic, stearic, palmitic, and those obtained from taloil or black liquor soap in wood pulp manufacture.

(8) Certain fatty acids and their mono- or di-glycerides such as wood soap fatty acids, glycerol mono-ricinoleate, di-glycerol oleate, etc. Sulfonated fatty acids may also be used.

(9) Sulfonated terpenes, and especially their polymerization products and their condensation products such as terpenyl phenol sulfonate, terpenyl naphthalene sulfonate, etc.

(10) Salts of phosphoric acid esters of higher alcohols or of phosphoric compounds of higher hydrocarbons.

(11) Salts of quaternary ammonium compounds such as the ester of lauric alcohol with chlorpyridino acetic acid.

Naturally, certain of the above surface active agents are more effective than are others for the emulsification of any given polybasic acid ester or mixture thereof, but all of the above classes of surface active agents possess emulsifying properties in greater or lesser degree. In Example 2 I have pointed out a representative composition which produces a stable emulsion, and this will serve to indicate the way in which the most suitable compositions can be prepared.

The invention will be further described in conjunction with the following specific examples, which are intended to illustrate typical compositions of the present invention and typical methods of applying them to the fibers. It should be understood, however, that these specific compositions are given by way of example, and not by way of limitation, and that where a component of one class of materials is used in conjunction with a component of another class this is intended as representative of the classes themselves. In other words, variations and substitutions of materials falling within the classes may be made without departing from the scope of the invention, which is limited only by the scope of the claims appended hereto.

## EXAMPLE 1

- Lubricants used in the textile industries are ordinarily evaluated on the basis of their lubricating qualities, their scouring qualities or completeness of removal from the thread or fabric after spinning or weaving by the ordinary detergent methods, their resistance to rancidity or oxidation and their physical and chemical constants.
- 10 The constants of greatest importance are their viscosity, their cold test, their flash point and their resistance to auto-oxidation or spontaneous combustion which is determined by the so-called Mackey test.
- 15 In the following examples, the new lubricants of the present invention will be described in detail with reference to the above properties. In order to exemplify the methods by which these properties are determined, the following tests
- 20 will be described in detail with reference to simple esters of phthalic acid, using two natural non-drying oils, teased oil and olive oil, as standards of comparison.

## FRICITION TESTS

- 25 To establish a standard of lubricating properties, the following tests were made:
- A 200 gram weight was attached to one end of a thread of 36/3 grey cotton, this material being chosen in preference to a wool thread by reason of its greater uniformity. The thread was impregnated with the lubricant under test and the excess lubricant removed by drawing the thread through two tightly clamped pieces of rubber.
- 30 The lubricated thread was then suspended over a glass rod and its free end was attached to a metal rod which was moved up and down by a series of pulleys and an electrically driven motor. The friction of the thread moving over the glass rod eventually caused rupture, and the time required for this rupture of the thread was automatically recorded by a stop watch. Check tests showed that the results obtained with this apparatus are easily and closely reproducible.
- 35 40 45 Synthetic esters having the following physical and chemical constants were tested in the above described apparatus:

TABLE 1.—Physical and chemical constants

| Lubricant                               | Viscosity | Cold test | Acid No. | Flash point |
|-----------------------------------------|-----------|-----------|----------|-------------|
| 55 Dimethyl phthalate.....              | ≤A        | ≤-30      | 1.2      | 142         |
| Diamyl phthalate.....                   | ≤A        | ≤-30      | 0.57     | 167         |
| Diethyl phthalate.....                  | A         | -30       | 1.4      | 193         |
| Dibutyl phthalate.....                  | ≤A        | ≤-30      | 0.57     | 165         |
| Dihexyl (methyl amyl) phthalate.....    | B-C       | ≤-30      | 2.3      | 164         |
| Dibutyl glycol diphthalate.....         | V         | 10        | 6.3      | 191         |
| 60 Dihexyl (ethyl butyl) phthalate..... | ≤A        | ≤-30      | 1.4      | 174         |
| Diethyl phthalate.....                  | ≤A        | ≤-30      | 1.0      | 161         |

<sup>1</sup> Viscous.<sup>2</sup> Solid.

- 65 As a comparison, a vegetable oil was used having the following constants:

| Lubricant          | Viscosity | Cold test    | Acid No. | Flash point |
|--------------------|-----------|--------------|----------|-------------|
| 70 Teased oil..... | C         | 1-15<br>≤-30 | 2.84     | 284         |

<sup>1</sup> Cloudy.<sup>2</sup> Solid.

The following table gives the time required to rupture the thread in the above described apparatus:

TABLE 2.—Friction tests

| Lubricant tested                | Time required to rupture thread |      |      |      |
|---------------------------------|---------------------------------|------|------|------|
|                                 | Min.                            | Sec. | Min. | Sec. |
| Dimethyl phthalate.....         | 6                               | 39   | 6    | 9    |
| Distilled diamyl phthalate..... | 12                              | 50   | 12   | 33   |
| Diethyl phthalate.....          | 12                              | 36   | 11   | 30   |
| Dibutyl phthalate.....          | 7                               | 30   | 7    | 45   |
| Dimethyl amyl phthalate.....    | 5                               | 13   | 5    | 20   |
| Dibutyl glycol diphthalate..... | 9                               | 30   | 9    | 55   |
| Diethyl butyl phthalate.....    | 7                               | 15   | 7    | 3    |
| Diethyl phthalate.....          | 35                              | 10   | 35   | 16   |
| Teased oil.....                 | 6                               | 57   | 7    | 18   |
| Olive oil.....                  | 4                               | 57   | 5    | 12   |

The tests indicated that diethyl phthalate was by far the best lubricant, and that diamyl and di-octyl phthalates were next. All the synthetic esters were superior in lubricating value to olive oil, which is a commonly used lubricant, and the majority of them were better than teased oil, which is one of the best textile lubricating oils. In view of the unusually high figure obtained with diethyl phthalate, the test with this material was repeated several times and the value obtained was found to be correct.

## SCOURING TESTS

Eighteen skeins of 36/3 grey cotton thread were prepared (allowing two for each ester tested) by the usual standard laboratory procedure. Each skein weighed approximately 5 grams. After drying the skeins for 2 hours at 110° C., they were weighed, tagged, and impregnated with the lubricant under test. Oiling was accomplished by immersing the skein in the oil or ester for 5 minutes and then allowing the oil to drip off the skein for 24 hours. The skeins were again placed into the oven for 2 hours at 70° C. and the quantity of the ester absorbed was determined from the difference in weight of each skein, before and after.

The skeins were placed into one pint screw cap jars containing 200 ccs. of water and 2½% of a 10% solution of sodium dioctyl sulfosuccinate, which is a wetting agent having good detergent properties. The amount of wetting agent was based on the weight of lubricant taken up by the skein. The jars were agitated for two hours at 60° C., after which the skeins were hung up to dry for 18 hours at room temperature and then for 2 hours at 70° C. The amount of the lubricant removed by washing was determined by the loss in weight of each skein. The results of these tests are given in Table 3.

TABLE 3.—Scouring tests

| Ester used for oiling                | Percent of ester removed by washing |      |
|--------------------------------------|-------------------------------------|------|
| Dimethyl phthalate.....              | 85.0                                | 84.3 |
| Diamyl phthalate.....                | 54.4                                | 54.5 |
| Diethyl phthalate.....               | 51.9                                | 52.3 |
| Dibutyl phthalate.....               | 63.5                                | 63.5 |
| Dihexyl (methyl-amyl) phthalate..... | 64.3                                | 67.5 |
| Dibutyl glycol diphthalate.....      | 70.0                                | 70.0 |
| Dihexyl (ethyl butyl) phthalate..... | 65.5                                | 64.2 |
| Diethyl phthalate.....               | 83.1                                | 83.1 |
| Teased oil.....                      | 48.4                                | 48.3 |

From the above it is seen that all the phthalic esters were washed out more easily and more

completely than the teaseed oil. Dimethyl phthalate and diethyl phthalate appear to possess the best scouring properties.

##### 5 ACCELERATED OXIDATION TESTS

In order to determine the degree of resistance to oxidation, thickening and rancidity upon storage of the lubricants of the present invention they 10 were subjected to an accelerated aging test in the presence of ultra violet light. The procedure was as follows:

Cotton strips of 5x12" were extracted with ether to remove all the oil and each strip was 15 pregnant with 2% of its weight of the oil to be tested. This was accomplished by dissolving the determined amount of oil or ester in 20 ccs. of ether and pouring the ether solution over the cloth in an evaporating dish, followed by evaporation of the ether. The samples of treated cloth 20 were then placed on asbestos boards of 5x12" and covered with black masking paper, allowing 3" of the cloth to remain exposed. The samples were then exposed to the light of a mercury arc 25 lamp in an atmosphere saturated with water vapor at 120° F. for 72 hours. 3" of masking were removed and the cloth was again exposed to the ultra violet rays for another 24 hours. Another 3" were removed and a further 24 hours 30 exposure was given. The changes in color of the treated samples were then noted and recorded as follows:

TABLE 4.—Accelerated aging test

| Lubricant                       | Color after exposure        |
|---------------------------------|-----------------------------|
| Dimethyl phthalate              | No change in color.         |
| Diethyl phthalate               | Very slight coloration.     |
| Diethyl phthalate               | Do.                         |
| Diethyl phthalate               | Do.                         |
| Dihexyl (methyl amyl) phthalate | Do.                         |
| Diethyl glycol diphtalate       | Slight coloration.          |
| Dihexyl (ethyl butyl) phthalate | Very slight coloration.     |
| Diethyl phthalate               | No change in color.         |
| Teaseed oil                     | Distinct yellow coloration. |

45 From the above, it is seen that the phthalic esters are practically unaffected by ultra violet rays as compared with non-drying vegetable oils.

##### 50 MACKEY TEST

A description of this test, and of the apparatus used in performing it, is given in Allen's "Commercial Organic Analysis," Fifth Edition, volume 55 No. 2, pages 759-761, and the values obtained with standard vegetable oil lubricants are stated. The neutral esters of phthalic acid, being completely stable, showed no temperature rise even on prolonged heating for 4-5 hours. This means that 60 these esters present no fire hazard upon storage of the oiled or lubricated threads or fabrics.

##### EXAMPLE 2

65 The oiling of wool is usually performed during the "mixing," in which two or more grades or colors are blended. The wool is spread out on a floor or table and layers of the different grades are sprayed as the mix is made up. In 70 the most modern mills this is done by spraying the oil in the form of an emulsion through automatic sprayers in connection with the mixing picker.

75 For satisfactory results it is necessary to have a stable emulsion, and it is an advantage of the

esters of the present invention that they can be readily emulsified with emulsifying agents that will also promote their removal from the yarn or cloth in a subsequent scouring or washing step. Such an emulsion should contain, in addition to the lubricant and water, an emulsifying agent of the sulfonic acid type and an emulsion stabilizer such as lecithin, gum arabic, casein and the like. A typical emulsion of this type will have the following composition, the parts being by weight:

|                               | Parts   |
|-------------------------------|---------|
| Lubricant                     | 50      |
| Sodium dioctyl sulfosuccinate | 0.2-1.0 |
| Lecithin                      | 0.5-1.0 |
| Water                         | 50      |

Such a mixture can be easily emulsified with an ordinary high speed mechanical agitator and will remain stable indefinitely.

Instead of the sodium dioctyl sulfosuccinate in the above composition, 0.5-1.0 parts of sodium isopropyl naphthalene sulfonate, or of pinene phenol sulfonate, or of a higher fatty alcohol sulfate, or 0.5-2.0 parts of a highly sulfonated oil such as castor oil may be used.

##### EXAMPLE 3

In addition to their valuable properties when used alone, the esters of the present invention are well suited for use in admixture with the natural vegetable oils for the lubrication of wool, cotton, silk and other textiles. For example, they may be used in admixture with olive oil, coconut oil, palm oil, castor oil and the like as well as with modified oils such as Turkey red oil, sulfonated olive oil, sulfonated castor oil, etc. The mixture may also contain mineral oil, although this should not be present in so great a proportion as to prevent ready removal by scouring.

The improvements resulting from the admixture of esters of phthalic acid with castor oils is shown by the following tables. Castor oil is used as a softener in the dyeing and finishing of cotton piece goods. It is also the base of most of the oil mordants used in printing and dyeing. Mixtures of castor oil with the esters of organic dicarboxylic acids of the present invention may be substituted for straight blown or unblown castor oil in any of these applications.

TABLE 1

| Ester of phthalic acid used | Grams of ester | Grams of unblown castor oil | Grams of blown castor oil | Viscosity | Acid number |
|-----------------------------|----------------|-----------------------------|---------------------------|-----------|-------------|
| Dimethyl                    | 150            | 120                         | —                         | A-B       | 4.2         |
| Do                          | 150            | —                           | 50                        | A-B       | 6.8         |
| Diethyl                     | 150            | 160                         | —                         | A-B       | 4.9         |
| Do                          | 150            | —                           | 50                        | A-B       | 8.6         |
| Dibutyl                     | 150            | 100                         | —                         | A-B       | 3.9         |
| Do                          | 200            | —                           | 50                        | A-B       | 6.8         |
| Diethyl                     | 175            | 50                          | —                         | A-B       | 3.5         |
| Do                          | 210            | —                           | 50                        | A-B       | 6.3         |
| Oils                        |                |                             |                           |           | 60          |
| Castor oil                  |                |                             |                           | U         | 10.3        |
| Blown castor oil            |                |                             |                           | >25       | 17.8        |
| Teaseed oil                 |                |                             |                           | O         | 2.8         |
| Olive oil                   |                |                             |                           | B-C       | 1.2         |

Solidifying points, flash points, influence of ultra violet irradiation, lubricating and scouring properties, are given in Table 2.

TABLE 2

| 5  | Lubricant used                      | Cold test, °C. | Flash point, °C. | Color after ultraviolet irradiation | Time required to rupture thread | Percent oil removed on scouring |
|----|-------------------------------------|----------------|------------------|-------------------------------------|---------------------------------|---------------------------------|
| 10 | Dimethyl phthalate—castor oil       | <-30           | 146              | 2                                   | 5 32                            | 67.2                            |
|    | Dimethyl phthalate—blown castor oil | <-30           | 147              | 2                                   | 6 12                            | 64.8                            |
|    | Diethyl phthalate—castor oil        | <-30           | 157              | 3                                   | 9 30                            | 66.1                            |
|    | Diethyl phthalate—blown castor oil  | <-30           | 156              | 3                                   | 8 30                            | 58.3                            |
|    | Dibutyl phthalate—castor oil        | <-30           | 174              | 2                                   | 6 45                            | 58.6                            |
| 15 | Dibutyl phthalate—blown castor oil  | <-30           | 171              | 2                                   | 5 59                            | 54.9                            |
|    | Diamyl phthalate—castor oil         | <-30           | 183              | 2                                   | 4 12                            | 49.6                            |
|    | Diamyl phthalate—blown castor oil   | <-30           | 175              | 2                                   | 4 34                            | 49.5                            |
|    | Castor oil                          | -18            | 273              | 7                                   | 4 30                            | 45.7                            |
|    | Blown castor oil                    | 3              | 198              | 4                                   |                                 |                                 |
| 20 | Teased oil                          | -30            | 284              | 6                                   | 6 59                            | 42.1                            |
|    | Olive oil                           | -8             | 304              | 5-6                                 | 4 15                            | 43.3                            |
|    | Blank                               |                |                  | 1                                   | 3 20                            |                                 |

<sup>1</sup> Diethyl phthalate used in this experiment had a flash point of 152° C. as compared with 161° C. for diethyl phthalate from a different source used in previous experiments.

<sup>2</sup> In evaluation of stability to ultraviolet irradiation, 1 means best and 7 means worst in the series.

From the above it will be noted that diethyl phthalate will more than double the lubricating value of castor oil when mixed with it in equal quantities and that it improves the scouring properties, the cold test, and other figures. Dimethyl and dibutyl phthalates produce the second best results, while improvements in the cold test and scouring properties are shown by all the esters.

Each of the above mixtures, when subjected to the Mackey test, showed no temperature rise even after several hours heating. Accordingly, textiles lubricated with these mixtures are completely stable upon storage and will present no spontaneous combustion hazard.

The color of cotton cloth impregnated with the above mixtures and exposed to ultraviolet light as in Example 1 indicated that they show much less discoloration than castor oil, blown castor oil, teased oil or olive oil. Cloth impregnated with castor oil alone became considerably darker after irradiation and developed a distinct odor of rancidity.

The use of the esters of the present invention in admixture with other standard lubricants of natural origin is shown by the following.

TABLE 3

| 55 | Composition                        | Viscosity | Acid number | Flash point | Cold test                        | Color after radiation | Lubrication time required to rupture thread | Percent oil removed on washing | Color of oil |
|----|------------------------------------|-----------|-------------|-------------|----------------------------------|-----------------------|---------------------------------------------|--------------------------------|--------------|
| 60 | Olive oil, 33.3 grams              | 15 sec.   | .89         | 171         | {-22° C. cloudy, -30° C. solid}  | 1                     | 4 48                                        | 45.45                          | <1L          |
|    | Dibutyl phthalate, 66.7 grams      | 15.9 sec. | .75         | 175         | {-30° C. cloudy, -30° C. solid}  | 2                     | 6 38                                        | 37.45                          | <1L          |
|    | Olive oil, 33.3 grams              | A         | 6.3         | 203         | Solid at 12° C.                  | 1                     | 4 10                                        | 35.0                           | 1            |
|    | Diamyl phthalate, 66.7 grams       | 16 sec.   | .89         | 101         | {-20° C. cloudy, <-30° C. solid} | 1                     | 4 02                                        | 21.2                           | 1L           |
| 65 | Coconut oil                        |           |             |             |                                  |                       |                                             |                                | 65           |
|    | Olive oil, 33.3 grams              | 15 sec.   | .89         | 171         | {-5° C. cloudy, -30° C. solid}   | 1                     | 5 12                                        | 52.5                           | 1            |
|    | Gulfgem oil B, 66.7 grams          | 15.8 sec. | 2.51        | 171         | Solid at -25° C.                 | 1                     | 6 32                                        | 50.2                           | 2            |
|    | 1.25 gms. lard                     | A         | 5.64        | 173         | {+10° C. cloudy, -15° C. solid}  | 1                     | 4 20                                        | 52.7                           | <1L          |
|    | 50 gms. dibutyl glycol diphthalate |           |             |             |                                  |                       |                                             |                                | 70           |
|    | 150 gms. dibutyl phthalate         |           |             |             |                                  |                       |                                             |                                |              |
|    | 12.5 gms. gulfgem oil B            |           |             |             |                                  |                       |                                             |                                |              |
|    | 1.25 gms. lard                     |           |             |             |                                  |                       |                                             |                                |              |
|    | 50 gms. dibutyl glycol diphthalate |           |             |             |                                  |                       |                                             |                                |              |
| 70 | 70 gms. dibutyl phthalate          |           |             |             |                                  |                       |                                             |                                |              |
|    | 100 gms. coconut oil               |           |             |             |                                  |                       |                                             |                                |              |
|    | 30 gms. dibutyl glycol diphthalate |           |             |             |                                  |                       |                                             |                                |              |
|    | 230 gms. dibutyl phthalate         |           |             |             |                                  |                       |                                             |                                |              |

NOTE.—Viscosities determined with Ford cup No. 4. Color determined by the Klett scale.

A=19.8 sec.

B=23.6 sec.

Gulfgem oil B is a low viscosity mineral oil with a flash point of 160° C., and is frequently added to textile lubricants.

The above figures show that the properties of olive oil are definitely improved by the addition of the synthetic esters of the present invention. They also show that such cheap materials as coconut oil and lard can be mixed with the synthetic esters to produce a lubricant having properties as good or better than olive oil. This is the case even when the lubricants are diluted with substantial amounts of mineral oil.

#### EXAMPLE 4

Esters of organic dicarboxylic acids with polyhydric alcohols, by reason of their relatively higher viscosity, are better suited for use as textile lubricants in admixture with oils or with esters of monohydric alcohols. When so used they greatly improve the cold test and Mackey test of these materials and their stability against discoloration. A few representative complex esters of polyhydric alcohols are the following:

TABLE 1

|                                     | Viscosity | Acid number | Cold test |
|-------------------------------------|-----------|-------------|-----------|
| Glycol oleate phthalate, 2 mols.    | O         | 10.5        | -25       |
| Teased oil, 1 mol.                  |           |             | 45        |
| Glycol glyceryl mono-phthalate, 50% | E         | 5.7         | -30       |
| Teased oil, 50%                     |           |             |           |
| Glycol phthalate oleate, 1 mol.     | G         | 5.7         | -20       |
| Dioleyl phthalate glyceride, 1 mol. |           |             |           |

TABLE 3

| 55 | Composition                        | Viscosity | Acid number | Flash point | Cold test                        | Color after radiation | Lubrication time required to rupture thread | Percent oil removed on washing | Color of oil |
|----|------------------------------------|-----------|-------------|-------------|----------------------------------|-----------------------|---------------------------------------------|--------------------------------|--------------|
| 60 | Olive oil, 33.3 grams              | 15 sec.   | .89         | 171         | {-22° C. cloudy, -30° C. solid}  | 1                     | 4 48                                        | 45.45                          | <1L          |
|    | Dibutyl phthalate, 66.7 grams      | 15.9 sec. | .75         | 175         | {-30° C. cloudy, -30° C. solid}  | 2                     | 6 38                                        | 37.45                          | <1L          |
|    | Olive oil, 33.3 grams              | A         | 6.3         | 203         | Solid at 12° C.                  | 1                     | 4 10                                        | 35.0                           | 1            |
|    | Diamyl phthalate, 66.7 grams       | 16 sec.   | .89         | 101         | {-20° C. cloudy, <-30° C. solid} | 1                     | 4 02                                        | 21.2                           | 1L           |
| 65 | Coconut oil                        |           |             |             |                                  |                       |                                             |                                | 65           |
|    | Olive oil, 33.3 grams              | 15 sec.   | .89         | 171         | {-5° C. cloudy, -30° C. solid}   | 1                     | 5 12                                        | 52.5                           | 1            |
|    | Gulfgem oil B, 66.7 grams          | 15.8 sec. | 2.51        | 171         | Solid at -25° C.                 | 1                     | 6 32                                        | 50.2                           | 2            |
|    | 1.25 gms. lard                     | A         | 5.64        | 173         | {+10° C. cloudy, -15° C. solid}  | 1                     | 4 20                                        | 52.7                           | <1L          |
|    | 50 gms. dibutyl glycol diphthalate |           |             |             |                                  |                       |                                             |                                | 70           |
|    | 150 gms. dibutyl phthalate         |           |             |             |                                  |                       |                                             |                                |              |
|    | 12.5 gms. gulfgem oil B            |           |             |             |                                  |                       |                                             |                                |              |
|    | 1.25 gms. lard                     |           |             |             |                                  |                       |                                             |                                |              |
|    | 50 gms. dibutyl glycol diphthalate |           |             |             |                                  |                       |                                             |                                |              |
| 70 | 70 gms. dibutyl phthalate          |           |             |             |                                  |                       |                                             |                                |              |
|    | 100 gms. coconut oil               |           |             |             |                                  |                       |                                             |                                |              |
|    | 30 gms. dibutyl glycol diphthalate |           |             |             |                                  |                       |                                             |                                |              |
|    | 230 gms. dibutyl phthalate         |           |             |             |                                  |                       |                                             |                                |              |

The results of tests outlined in Example 1 are as follows:

TABLE 2

| 5  | Lubricant                            | Flash point, °C. | Color after irradiation | Time required to rupture thread | Percent oil removed on scouring |
|----|--------------------------------------|------------------|-------------------------|---------------------------------|---------------------------------|
|    | Glycol oleate phthalate, 2 mols.     | 237              | 3                       | Min. 5 Sec. 18                  | 40.9                            |
| 10 | Teaseed oil, 1 mol.                  |                  |                         |                                 |                                 |
|    | Glycol glyceryl mono-phthalate, 60%. | 262              | 1                       | 4 18                            | 40.7                            |
|    | Teaseed oil, 60%.                    |                  |                         |                                 |                                 |
| 15 | Glycol phthalate oleate, 1 mol.      |                  |                         |                                 |                                 |
|    | Dioleyl phthalic glyceride, 1 mol.   | 258              | 2                       | 6 50                            | 54.0                            |
|    | Teaseed oil.                         |                  |                         |                                 |                                 |
|    | Olive oil.                           | 284<br>304       | 7<br>6-7                | 6 52<br>4 15                    | 40.0<br>43.3                    |

TABLE 1

| 20 | Composition                                                             | Viscosity | Acid number | Flash point | Cold test                     | Color after irradiation           | Lubrication value | Percent oil removed on washing | Color of oil |
|----|-------------------------------------------------------------------------|-----------|-------------|-------------|-------------------------------|-----------------------------------|-------------------|--------------------------------|--------------|
|    | 30 pts.—1mol diglycol phthalate oleate+1mol dioleyl phthalic glyceride. | 15.5 sec. | 2.3         | °C.<br>168  | {Cloudy—6°C.<br>Solid—17°C.}  | 2                                 | Min. Sec.<br>7 50 | 67.5                           | <1L          |
| 25 | 70 pts.—dibutyl phthalate.                                              |           |             | 16.1 sec.   | 1.7                           | 172 {Cloudy—10°C.<br>Solid—16°C.} | 2 8 12            | 62.7                           | <1L          |
|    | 20 pts.—1mol diglycol phthalate oleate+1mol dioleyl phthalic glyceride. |           |             |             |                               | {Cloudy—10°C.<br>Solid—16°C.}     | 2 4 09            | 63.2                           | <1L          |
|    | 80 pts.—dibutyl phthalate.                                              |           |             |             |                               | {Cloudy—10°C.<br>Solid—16°C.}     | 2 5 0             | 61.1                           | <1L          |
|    | 5 pts.—mono-lauryl ester of glycol.                                     |           |             |             |                               | {Liquid—30°C.}                    |                   |                                |              |
|    | 95 pts.—dibutyl phthalate.                                              | 13.1 sec. | 1.9         | 169         | {Cloudy—5°C.<br>Liquid—30°C.} | 2 5 0                             | 61.5              |                                |              |
|    | 5 pts.—mono-lauryl ester of glycol.                                     |           |             |             |                               | {Cloudy—5°C.<br>Liquid—30°C.}     |                   |                                |              |
|    | 95 pts.—diethyl phthalate.                                              | 13.5 sec. | 2.5         | 164         | {Cloudy—5°C.<br>Liquid—30°C.} | 2 5 0                             |                   |                                |              |
| 30 | 55 pts.—dimethoxy phenoxy ethyl fumarate.                               |           |             |             |                               | {Cloudy—5°C.<br>Liquid—30°C.}     |                   |                                |              |
|    | 50 pts.—dibutyl phthalate.                                              | A         | 2.1         | 176         | Clear <—30°C.                 | 1 7 58                            |                   |                                | 2 30         |

Note.—1 means best color and 7 means worst color. These results show the remarkable improvement in stability against rancidity and discoloration that is obtained when the esters of organic polycarboxylic acids with polyhydric alcohols are admixed with vegetable oils such as teaseed oil and olive oil.

#### EXAMPLE 5

The scouring properties of the lubricants of the present invention can be improved by incorporating therein an excess of hydroxy groups over and above those necessary for esterification of the di- or polycarboxylic acids used in their preparation. These excess hydroxy groups may be present in uncombined form as, for example, in the mono-acid esters of glycol or glycerol, or they may be esterified with monobasic acids such as oleic acid, ricinoleic acid, or other acids resulting from the saponification of coconut oil, olive oil, palm oil, teaseed oil or other similar vegetable oils. Such compounds can easily be prepared by reacting the natural fats or oils with excess glycerine to form the mono- or diglyceride,

which is then esterified with the di- or polycarboxylic acid. Similarly, in the case of esters of aromatic alcohols or phenols, the excess hydroxy groups may be attached to the aromatic nucleus as for example in dimethoxy phenoxy ethyl maleate or fumarate. In some cases ether groups will serve the same purpose, an example of this being the diethylene glycol phthalate resin described in Example 6 as Resin B.

A simpler method of improving the scouring value is to use the polyhydric alcohol esters in admixture with esters of mono-hydric alcohols that already have good scouring values. Table 1 shows the results obtained when the two methods are combined.

#### EXAMPLE 6

In addition to the simple physical admixture of the esters of the present invention with non-drying oils, as illustrated in Example 3, it is possible to utilize these materials in chemical combination with each other in the form of oil modified resins. This constitutes an important feature of the present invention because the tendency of many of the natural oils to discolor and to ignite spontaneously upon storage of the lubricated textiles is thereby overcome. In other words a lubricant such as castor oil which discolors badly (see Example 3, Table 2) becomes almost completely resistant to discoloration when used in the form of a long oil alkyd resin.

For example, a castor oil modified alkyd resin of 1000 oil length is prepared by heating together 148 parts of phthalic anhydride, 100 parts glycerol and 1000 parts of castor oil. The temperature is raised over a period of two hours to 200° C. with continuous agitation in an atmosphere of carbon dioxide and held at this figure for 7 hours or until an acid number of 3.6 is obtained. In Table 1 this is designated as Resin A. The results obtained are as follows:

TABLE 1

| 60 | Composition                                        | Viscosity | Acid number | Flash point | Cold test                                 | Color after irradiation | Lubrication value | Percent oil removed on washing | Color of oil |
|----|----------------------------------------------------|-----------|-------------|-------------|-------------------------------------------|-------------------------|-------------------|--------------------------------|--------------|
|    | 61 pts.—resin A.                                   |           |             |             |                                           |                         |                   |                                |              |
| 65 | 182 pts.—dibutyl phthalate.                        | A         | 2.4         | 173         | {v. viscous at —5° C.<br>Waxy at —12° C.} | 3 8 12                  | 73.0              | 1L                             | 65           |
|    | 10 pts.—di-stearyl di-glyceryl mono-phthalate.     |           |             |             |                                           |                         |                   |                                |              |
|    | 62 pts.—resin A.                                   |           |             |             |                                           |                         |                   |                                |              |
|    | 188 pts.—dibutyl phthalate.                        | A         | 1.0         | 173         | {v. viscous at —5° C.<br>Waxy at —10° C.} | 3 7 15                  | 64.3              | 1L                             |              |
|    | 10 pts.—di-(glyceryl monostearate) mono-phthalate. |           |             |             |                                           |                         |                   |                                |              |
|    | 60 pts.—resin A.                                   |           |             |             |                                           |                         |                   |                                |              |
| 70 | 150 pts.—dibutyl phthalate.                        | A         | 2.3         | 173         | Clear liquid at —15° C.                   | 4 6 52                  | 68.5              | 1L                             | 70           |
|    | 10 pts.—cyclohexanol stearate.                     |           |             |             |                                           |                         |                   |                                |              |
|    | 60 pts.—resin A.                                   |           |             |             |                                           |                         |                   |                                |              |
|    | 140 pts.—dibutyl phthalate.                        | B         | 1.5         | 173         | Waxy at —15° C.                           | 2 7 12                  | 84.6              | 1L                             |              |
|    | 5 pts.—sodium dioctyl sulfosuccinate.              |           |             |             |                                           |                         |                   |                                |              |
|    | 60 pts.—resin A.                                   | B         | 1.3         | 1           | Waxy at —18° C.                           | 1 6 51                  | 58.7              | 1L                             |              |
|    | 140 pts.—dibutyl phthalate.                        |           |             |             |                                           |                         |                   |                                |              |

75 Note.—Sodium dioctyl sulfosuccinate combines the properties of a lubricant and a wetting agent.

The last two columns of Table 1 illustrate another feature of the invention, namely, the use of esters of sulfonated dicarboxylic acids. A comparison of the figures will show that the addition of only 2.5% of such an ester will increase the scouring value enormously, and will also improve the lubricating properties of the composition.

Instead of castor oil, other lubricants of natural origin may be employed in the form of oil modified resins. A coconut oil modified alkyl resin giving good results may be prepared as follows:

A mixture of 203 parts phthalic anhydride, 154 parts diethylene glycol and 1375 parts coconut oil are heated during 1½ hours to 220° C. in an atmosphere of CO<sub>2</sub> and held for an acid number of 30. 90 parts of N-butyl carbinol are added and the temperature maintained at 180–210° C. for 13 hours after which time a resin having an acid number of 17 is obtained. In Table 2 this is designated as Resin B.

The use of resins containing less oil is illustrated by the following formulation:

148 parts phthalic anhydride, 80 parts glycerol and 200 parts castor oil are reacted over the same cooking schedule as Resin A in an atmosphere of CO<sub>2</sub>. The product has an acid number of 8 and a viscosity of V–V in 50% xylol solution. In Table 2 it is designated Resin C.

tion; they have no tendency toward spontaneous combustion and present no fire hazard when textiles lubricated with them are stored.

What I claim is:

1. A method of lubricating textiles which comprises contacting them with a lubricant comprising an ester of phthalic acid with a monohydric alcohol and a member of the class consisting of non-drying higher fatty acids and glycerides of non-drying higher fatty acids.

2. A method of lubricating textiles which comprises contacting them with a lubricant comprising an ester of an aromatic polycarboxylic acid selected from the group consisting of phthalic acid, phthalic anhydride, substituted phthalic acid and substituted phthalic anhydride with a monohydric alcohol.

3. A method of lubricating textile filaments which comprises contacting them with a lubricant containing a resin comprising the reaction product of phthalic anhydride, a polyhydric alcohol, and a quantity of a non-drying oil greater than the amount of the other two constituents.

4. A method of lubricating textile filaments which comprises contacting them with a lubricant containing a polyhydric alcohol ester of an organic polycarboxylic acid together with a monohydric alcohol ester of a phthalic acid.

5. A method of lubricating textiles which comprises contacting them with a lubricant contain-

TABLE 2

| 35                             | Composition               | Viscosity | Acid number | Flash point | Cold test                                | Color after irradiation | Lubrication value | Percent oil removed on washing | Color of Oil | 35 |
|--------------------------------|---------------------------|-----------|-------------|-------------|------------------------------------------|-------------------------|-------------------|--------------------------------|--------------|----|
| 30 pts.—resin B                |                           |           |             |             |                                          |                         |                   |                                |              |    |
| 40 70 pts.—dibutyl phthalate.  | 14.2 sec. Ford cup No. 4. | 5.7       | 170         | °C.         | {Cloudy -15° C<br>{Semi-solid -30° C     | 2                       | 5 33              | 50.1                           | 2L           | 40 |
| 20 pts.—resin B                | 14.5 sec. Ford cup No. 4. | 3.6       | 170         |             | {Cloudy -15° C<br>{Solid <-30° C         | 2                       | 5 37              | 62.9                           | 1L           |    |
| 80 pts.—diamyl phthalate.      |                           |           |             |             | {v. viscous -15° C<br>{Semi-solid -25° C | 3                       | 8 22              | 52.4                           | <1L          |    |
| 30 pts.—resin C                | T—U                       | 3.3       | 173         |             | do                                       | 2                       | 14 03             | 55.6                           | <1L          |    |
| 70 pts.—dibutyl phthalate.     |                           |           |             |             |                                          |                         |                   |                                |              |    |
| 20 pts.—resin C                |                           | 2.9       | 178         |             |                                          |                         |                   |                                |              |    |
| 80 pts.—diamyl phthalate.      |                           |           |             |             |                                          |                         |                   |                                |              |    |
| 50 pts.—resin C                |                           |           |             |             |                                          |                         |                   |                                |              |    |
| 45 200 pts.—dibutyl phthalate. | A                         | 2.9       | 174         |             | Clear and viscous -30° C                 | 1                       | 7 51              | 42.1                           | <1L          | 45 |

No Mackey test figures are shown in the above tables because none of the materials showed any temperature rise, even after prolonged heating. This is true of all the esters of the present inven-

ing the reaction product of a phthalic acid, a polyhydric alcohol, and a fatty acid.

50 ALPHONS O. JAEGER.